# EUROPEAN PATENT SPECIFICATION

(11) **EP 4 402 310 B1**
(45) Date of publication and mention of the grant of the patent: **30.04.2025**
(21) Application number: 22719341.4
(22) Date of filing: 29.03.2022
(51) Int. Cl.: D02G 3/28, D02G 3/44

(54) **WOOL LIKE YARN FOR CARPETS AND THE LIKE**
WOLLÄHNLICHES GARN FÜR TEPPICHE UND DERGLEICHEN
FIL DE TYPE LAINE POUR TAPIS ET ARTICLES SIMILAIRES

(30) Priority: 02.02.2022 IN 202221005619
(43) Date of publication of application: 24.07.2024
(73) Proprietor: AYM Syntex Ltd, 400013 Mumbai (IN)
(72) Inventor: MANDAWEWALA, Abhishek Rajesh, Mumbai 400025 (IN)
(74) Representative: Nederlandsch Octrooibureau
(86) International application number: PCT/IB2022/052877
(87) International publication number: WO 2023/148535

(56) References cited:
- EP-A1- 1 544 333
- WO-A1-2004/092462
- CN-A- 101 423 990

## Description

### TECHNICAL FIELD

The present disclosure generally relates to a method of manufacturing continuous filament yarn as a replacement of wool yarn for floor covering applications such as carpets and the like. The disclosure further relates to a wool-like yarn of continuous filament and to a floor covering manufactured from the yarn.

### BACKGROUND

Conventionally wool has remained a most preferred fibre for making carpet yarns due to its natural bulk, softness, resiliency and thermal behaviour. It is also popular for its natural origin and hairy or woolly structure.

Lately wool has lost its most preferred status in the floorcovering industry due mainly to the following perceived disadvantages.
1) As it must be collected from sheep or other animals by shearing, there has been an increase in animal rights activity seeking to stop or reduce the use of wool.
2) As wool fibres generally used in floorcovering application have fibre lengths of 60 - 200 mm, loss of fibres, often referred to as linting, from the wool yarn can be a health disadvantage as it can cause respiratory issues.
3) Wool yarn used in floorcovering applications is mostly non-recyclable, as recovery of long fibres from a floorcovering product is limited, due to breakage of fibres, making them much smaller in length and thus imposing greater risk of linting.

Additionally, the cost of wool is often considerably greater than synthetic alternatives, while their susceptibility to pests such as moths is well known.

To overcome the disadvantages of wool yarn in floorcovering application, bulked continuous filament (BCF) yarns made from polyester, polypropylene and nylon have gained popularity due to their continuous filament nature, that prevents linting, in addition to their reduced price. For these fibres, artificial bulk can be provided during the filament production process by texturizing the filaments e.g. by friction disc or stuffer box texturizing. They also exhibit good recyclability via mechanical or chemical recycling processes. CN-A-101 423 990 and WO-A-2004/092462 give examples of textured yarns that attempt to imitate natural yarns such as wool and cotton. A process of texturizing partially oriented yarn (POY) to produce fantasy yarns is disclosed in EP-A-1 544 333.

Nevertheless, the process of making BCF yarn for floorcovering application could never provide the feel and texture of products made from wool yarn due to the missing hairy look and feel of BCF yarn. Thus, a loop-pile floorcovering material produced from BCF or other textured continuous filaments was never able to provide the same natural hairy look and feel of products made from wool yarn.

Thus it would be desirable to produce a continuous filament yarn for floorcovering application, which could replace wool yarn by replicating its look, feel and hairiness with the additional advantage of being made from man-made fibre with low linting and good recyclability.

### SUMMARY

According to the invention, there is provided a method of manufacturing a wool-like yarn from continuous filaments of polymer material for use as an upstanding pile of a floor covering, wherein the yarn is obtained by a process comprising steps of: providing at least partially oriented, continuous filaments of the polymer; drawing and air texturizing the filaments to form a thread, wherein a first group of straight filaments forms a core of the thread and a second group of filaments are overfed with respect to the first group of filaments to form a hairy sheath; and twisting and/or cabling a plurality of threads together to form the wool-like yarn to have a weight of greater than 2000 dtex.

The resulting yarn exhibits a surprisingly similar look, feel and hairiness to that of wool yarn, while overcoming drawbacks of wool yarn such as linting, recyclability, UV resistance, antistatic properties and wear resistance.

Air texturizing of suitable polymer filaments has been shown to provide a useful degree of wooliness to the resulting yarn that exits the air texturizing process. For the purpose of the present invention, this yarn is referred to as a thread, to distinguish it from the subsequently assembled yarn of high dtex. It will nevertheless be understood that this is also a yarn, albeit of lower weight. As is otherwise conventional in air texturizing, air jets or the like cause the overfed filaments to entangle with one another to form a woolly or hairy envelope or sheath around the core. This sheath is sometimes referred to as the effect. Those filaments in the core that are not overfed are kept relatively straight and do not thus become entangled or are entangled to a lesser degree.

In the presently described process, the filaments may be initially provided in their partially oriented state. In consequence, they can be further drawn prior to the texturizing step. This can be used to remove nips or bonds between adjacent filaments or otherwise straighten them prior to the air texturizing process. They may be drawn to a fully oriented state or remain partially oriented in the final product. In preferred embodiments, the filaments have been drawn by at least 5% or at least 10% or at least 20% but less than 100%. It is also possible to use fully oriented yarns, since it is still possible to apply a limited amount of further drawing at the air texturizing stage, sufficient to break open any nips. It will be understood that fully drawn yarn may be drawn by more than 300%.

Twisting and/or cabling will take place in a subsequent step, which may take place at a different time and/or location to the air texturizing. In general, this will mean that the threads are wound to reels or bobbins. A number of reels will then be brought together for twisting. The reels may be provided with the same or different threads, e.g. of different colours. In the following, reference to twisting is intended to include cabling. In particular, in a first twisting step, a number of threads may be assembled together e.g. by light twisting to form a ply. In this context, twisting may also include air-twisting or false twisting, e.g. where alternate clockwise and anticlockwise twists are applied. Subsequently, a number of plies may be twisted or cabled together to form the wool-like yarn. By first assembling a number of threads together, high speed unwinding may be facilitated, whereby a cabling operation may proceed more quickly.

The filaments may be of any suitable weight according to the desired look and feel of the final product The filaments may all be of the same weight or some may be heavier than others. In an embodiment, heavier filaments may be provided in the sheath. Since certain air-texturising machines may be limited in the number of reels that can be combined, varying the weight of the respective filaments allows variation of the relative weights of the core and sheath. In an embodiment, the plurality of continuous filaments have a dtex per filament in a range from 0.5 dtex per filament to 10 dtex per filament. Preferably, these values lie in a range of 4 to 6 dtex per filament, which has been found to provide a more stable process with less risk of filament breakage.

Furthermore, the at least partially oriented, continuous filaments may be provided from any suitable source of such filaments. In particular, they may be produced on site at the same location or may have been produced elsewhere. They may be produced by any conventional process, in particular by melt spinning and drawing. It is also possible that the at least partially oriented, continuous filaments are provided as bulk continuous filaments (BCF). In this case, the filaments are already texturised and may be fully oriented. Using BCF has certain advantages over non-texturised filaments. Firstly, since initial texturizing increases their bulk, BCF has a higher weight and it is easier to achieve the required overall dtex value for the wool-like yarn. This may be important where the air-texturizing machine is limited by the number of reels at the input side. It also means that fewer threads may need to be assembled or twisted and the air texturizing step may operate more effectively. Furthermore, use of textured BCF for the filaments in the core of the thread can increase their entanglement with and grip on the filaments of the sheath.

The filaments may also have any suitable cross-sectional shape. In certain embodiments, the partially oriented, continuous filaments are of a multilobal cross-sectional shape. This can further enhance the similarity with wool, since filaments of non-circular cross-section can have a less shiny appearance than those having a smooth cross-section. In an embodiment, octolobal filaments may be used.

The at least partially oriented, continuous filaments may be provided as a plurality of multi-filament tows. Each tow may be presented on its own reel or bobbin as provided at the end of an extrusion process. Such tows are commonly referred to in the art as partially oriented yarn (POY) and are referenced here as tows, merely for the purpose of distinguishing these loosely bundled filaments from the resulting heavy weight wool-like yarn as the outcome of the overall process. Preferably the tow is provided with nips to hold each tow together. The skilled person will be familiar with such processes that allow the filaments within a tow to be held together. This may take place by air entanglement or other equivalent procedures. Each tow may comprise from 10 to 500 filaments, preferably between 100 and 200 filaments. Furthermore, each tow may have a dtex in a range of from 100 dtex to 1500 dtex, preferably from around 500 dtex to 700 dtex. The weight of each tow will depend on the production machinery that delivers the continuous filaments and also on the nature of the air-texturising machine to be used. It will be understood, that the intention is to produce thread having a relatively high dtex value and that this can be achieved either by having high dtex tows or by combining a greater number of tows during the air-texturising process. Where this process is limited by the number of reels that can be combined, it is advantageous to use high dtex tows. In an embodiment, the air texturising process is used to combine a number of such tows together, whereby a first tow forms a core of the thread and one or more further tows are overfed to form the hairy sheath. All of the tows may be identical or the tow or tows forming the core may be different from the tow or tows forming the sheath. As noted above, in cases where e.g. only two tows can be combined in an air texturizing machine, the tow forming the sheath may be of a higher dtex than the tow forming the core.

In an embodiment, drawing and air texturizing may takes place simultaneously in a continuous process. In this context, simultaneously is intended to mean that the tows are drawn prior to air texturizing in an inline process, without being subsequently wound to a bobbin. Drawing is particularly useful as a method of releasing the filaments in the tow for subsequent air texturizing. This can release any nip or connection between the filaments that might otherwise have impeded the air texturizing process. All of the filaments may be drawn to a fully oriented condition. Alternatively, only some of the filaments may be drawn and e.g. the filaments forming the core may be not further drawn and still nipped together. In an embodiment all of the filaments are drawn at a draw ratio of more than 1.3, preferably more than 1.5. Additionally, or in an alternative, the filaments of the sheath are drawn at a greater draw ratio than the core. In an embodiment, the filaments of the sheath are drawn at a ratio that is greater than that of the core to the same degree as they are overfed. This may result in a constant speed delivery of both groups of filaments.

The process of drawing and air texturizing may be performed in an otherwise conventional manner using conventional machinery. For polyester, drawing is preferably performed at a temperature around 180°C. The skilled person will be aware that this temperature may correspond to the normal temperature used during filament production for orienting the polymer. The filaments or tows may be subsequently cooled either before or during the air texturizing process.

During the air texturizing process, the degree of overfeeding may be determined according to the desired result. As the skilled person will understand, the degree of overfeeding will influence the volume of the sheath and hence the wooliness of the resulting thread. In an embodiment, the second group of filaments are overfed with respect to the first group of filaments by between 30% and 150%, preferably by around 80 %.

The properties of the thread will also be influenced by the ratio of the number of filaments in the core to the number of filaments in the sheath. In preferred embodiments, this ratio may be between 1:1 and 1:6, preferably around 1:2. For the case that the filaments in the core are distinct from those in the sheath, it is noted that it may be desirable that the ratio of the dtex of the core to the dtex in the sheath may also be between 1:1 and 1: 6, preferably around 1:2.

Depending upon the weight of the filaments and the number of filaments combined to form each thread, the thread may have a dtex in a range of from 500 dtex to 5,000 dtex. In general, threads at the lower end of this range are too light for floor covering applications. As discussed above, a heavyweight yarn can be produced by assembling a number of threads together. Preferably, from 2 to 20 threads may be assembled together by twisting and/or cabling to form the wool-like yarn. The resulting yarn will thus have a weight of greater than 2000 dtex but more generally will have a weight of greater than 5000 dtex or even greater than 10 000 dtex or up to 50 000 dtex. Preferably, the threads have a weight of between 2000 dtex and 3000 dtex.

The yarn may be lightly twisted or highly twisted. In general, it will be twisted in a range of from 30 to 400 twists per meter (TPM). As noted above, the yarn may be assembled in a multi-step process, whereby in a first step, groups of threads are twisted together as a ply and in a further step, two or more plies are twisted or cabled together.

The process may also comprise heat setting of the twisted yarn, preferably in a temperature range between 85°C - 200°C. This is especially desirable for highly twisted yarn of more than 100 TPM or more than 200 TPM in order to better maintain the twist during subsequent processing and use of the yarns and the subsequently manufactured floor covering. Heat setting preferably takes place at a temperature that is below the drawing temperature preferably in a temperature range between 85°C - 110°C.

The polymer material used to manufacture the continuous filaments may be any suitable polymer having the required properties for its use as a component in a floor covering. Typically, it may be selected from the group consisting of polyesters, polyamides, polypropylene and copolymers thereof. The invention is particularly applicable to polyesters including PET and PBT.

The invention also relates to a wool-like yarn for use as upstanding pile in the manufacture of floor coverings, the yarn comprising continuous filaments of polymer material assembled together to form threads with first straight filaments forming a core of the thread and second textured filaments forming a hairy sheath around the core and wherein a plurality of threads are twisted and/or cabled together to form a heavyweight yarn of greater than 2000 dtex. The yarn and its constituent threads and filaments may be as described above and hereinafter. In particular, the yarn may comprise filaments of the polymer combined with other fibres or filaments in a mixed yarn. The yarn may however alternatively consist essentially only of continuous filaments of a single polymer. In this sense, 'consists essentially' is intended to mean that the yarn is at least 99% or at least 95% of a single polymer filament. The remainder may be other fibres or filaments having particular functional purpose, such as anti-static conducting filaments, decorative or reflective filaments and the like .

Furthermore, the polymer of the wool-like yarn may include one or more masterbatches of additional materials mixed into the polymer. The masterbatches may be selected from the group consisting of anti-microbial, anti-fungal, UV resistant, FR, stain resistant, anti-oxidant and pigment or any other of the conventional masterbatches that the skilled person would contemplate adding to such filament. Furthermore, the yarn may be subjected to any conventional dye processes, such as the use of disperse dye for polyester or acid dye for nylon. Additionally, space dyeing may be used to create a variegated colour such as by hank dyeing or by bobbin dyeing.

The invention also relates to a floor covering comprising the wool-like yarn described above or hereinafter. In preferred embodiments, the floor covering is a carpet or rug. The wool-like yarn forms an upstanding pile, which may be a cut-pile, a loop-pile, a shag-pile or the like.

The wool-like yarn may be tufted, knitted, knotted and/or woven into the floor covering. It may also form the backing of the floor covering or the backing may be formed separately of another material.

### BRIEF DESCRIPTION OF THE DRAWINGS

The features and advantages of the present disclosure will be appreciated upon reference to the following drawings of an exemplary embodiment, in which
Figure 1 shows in schematic view, the four steps of a method according to the invention;
Figure 2 shows a cross-section through the yarn produced according to the method of Figure 1; and
Figure 3 shows a loop-pile tufted carpet incorporating the yarn produced according to the method of Figure 1.

### DESCRIPTION

The following detailed description illustrates an embodiment of the present disclosure and ways in which they can be implemented. Although some modes of carrying out the present disclosure have been disclosed, those skilled in the art would recognise that other embodiments for carrying out or practising the present disclosure are also possible.

Figure 1 shows the steps of a method for manufacturing a wool-like yarn according to an exemplary embodiment of the invention.

In a first step, according to Figure 1A, a plurality of continuous filaments 1 of polyester are extruded from an extruder 10 and drawn over rollers 20 in an otherwise conventional process for making partially oriented yarn (POY). The filaments 1 are spin-drawn at a draw ratio of 1.05 to have a weight of 6 dtex per filament. In total, 96 filaments 1 are wound together as a tow 2 to a reel 3. Prior to winding, the tow 2 is impinged by an intermingling jet 30 to nip the tow 2 together by slightly intermingling the individual filaments 1.

In a second step shown in Figure 1B, three reels 3, each wound with a tow 2 of continuous polyester filaments 1, are combined together and texturised in an air texturizing machine 40. The air texturizing machine 40 is an otherwise standard machine available from SSM. The tows 2 are first drawn through a drawing station 42 at a draw ratio of 1.7 and at a temperature of 180°C prior to delivery to the air texturizing station 44. In the air texturizing station 44, two of the tows 2 are overfed by an amount of 80% with respect to the third tow 2. Texturising jets 46 of air are applied to the tows 2, causing the overfed tows 2 to billow and form loops with respect to the third tow 2 which remains relatively straight. The overfed tows 2 thus form a hairy sheath 4 or effect around the third tow 2, which forms a core 12. The combined tows 2 at the exit of the air texturizing machine 40 form a thread 5, with a weight of 1480 dtex, which is wound to a bobbin 6.

In a third step, shown in Figure 1C, four bobbins 6 carrying air-texturised thread 5 are lightly wound together to form a ply 7. The ply has a weight of 6000 dtex and is wound with a twist of 80 tpm to a spool 8.

In a fourth step, shown in Figure 1D, two plies 7 are twisted together to form a wool-like yarn 9, having a weight of 12000 dtex. The plies 7 are twisted at 100 tpm. Figure 2 shows a cross-section through the yarn 9 of Figure 1D, illustrating the two plies 7. Each of the plies 7 is formed of four threads 5. The threads 5 exhibit a core 12 and a surrounding sheath 4, each composed of filaments 1.

Figure 3 shows a loop-pile tufted carpet 20. The carpet 20 has a woven backing 22, into which are tufted yarns 9 as illustrated in Figures 1 and 2. The yarns 9 form upstanding loops 24.

### Example 1

A yarn 9 as described above in relation to Figures 1A-D is employed in the manufacture of a tufted loop-pile carpet as shown in Figure 3. The carpet is tufted at ¼ inch gauge (6 mm) with 28 stitches per 10cm . The pile had a height of 10 mm. The resulting carpet appeared wool-like in all aspects and had a woolly appearance and touch.

The carpet was subjected to Hexapod testing. After 4000 cycles, the carpet exhibited a Hexapod rating of 4.5, which decreased to 4 after 8000 cycles and remained at 4 after 12000 cycles.

Thus, the invention has been described by reference to certain examples discussed above. It will be recognized that these embodiments are susceptible to various modifications and alternative forms well known to those of skill in the art. In particular, different initial filament weights may be employed according to the intended use. Many modifications in addition to those described above may be made to the structures and techniques described herein without departing from the scope of the invention. Accordingly, although specific embodiments have been described, these are examples only and are not limiting upon the scope of the invention as defined in the claims.

## Claims

1. A method of manufacturing a wool-like yarn (9) from continuous filaments (1) of polymer material for use as an upstanding pile of a floor covering (20), wherein the yarn is obtained by a process comprising steps of:
- providing at least partially oriented, continuous filaments of the polymer;
- drawing and air texturizing the filaments to form a thread (5), wherein a first group of straight filaments forms a core (12) of the thread and a second group of filaments are overfed with respect to the first group of filaments to form a hairy sheath (4);
- twisting and/or cabling a plurality of threads together to form the wool-like yarn (9) having a weight of greater than 2000 dtex.

2. The method as claimed in claim 1, wherein the plurality of continuous filaments have a dtex per filament value in a range from 0.5 to 10, preferably from 4 to 6 and/or are provided by melt spinning and drawing and/or are of a multilobal cross-sectional shape.

3. The method of any one of the preceding claims, wherein the partially oriented, continuous filaments are provided as a plurality of multi-filament tows (2), each preferably having a dtex in a range of from 100 dtex to 1500 dtex and preferably provided with nips to hold each tow together, wherein a first tow forms a core of the thread and at least one further tow is overfed to form the hairy sheath.

4. The method of any one of the preceding claims, wherein drawing and air texturizing takes place simultaneously in a continuous process.

5. The method of any one of the preceding claims, wherein drawing is performed at a temperature in a range of 130°C - 200°C.

6. The method of any one of the preceding claims, wherein the second group of filaments are overfed with respect to the first group of filaments by between 30% and 150%, preferably around 80%.

7. The method of any one of the preceding claims, wherein a dtex weight ratio of the filaments in the core to the filaments in the sheath is between 1:1 and 1:6, preferably 1:2.

8. The method of any one of the preceding claims, wherein the thread has a dtex in a range of from 500 dtex to 5000 dtex, preferably 2000 dtex to 3000 dtex.

9. The method of any one of the preceding claims, wherein from 2 to 20 threads are twisted and/or cabled together to form the wool-like yarn and/or the twisted and/or cabled yarn is twisted in a range of from 30 - 400 twists per meter (TPM).

10. The method of any one of the preceding claims further comprising heat setting of the twisted and/or cabled yarn to maintain the twist at a temperature below the drawing temperature, preferably in a temperature range between 85°C - 110°C.

11. The method of any one of the preceding claims, wherein the polymer is selected from the group consisting of polyesters, polyamides, polypropylene and copolymers thereof, preferably polyester, and/or the yarn consists of at least 99% or at least 95% of filaments of a single polymer.

12. A wool-like yarn (9) for use as upstanding pile in the manufacture of floor coverings (20), the yarn comprising continuous filaments (1) of polymer material, assembled together to form threads (5) with first straight filaments forming a core (12) of the thread and second textured filaments forming a hairy sheath (4) around the core and wherein a plurality of threads are twisted and/or cabled together to form a heavyweight yarn of greater than 2000 dtex.

13. The wool-like yarn of claim 12, wherein the polymer material includes one or more masterbatches, selected from the group consisting of: anti-microbial, anti-fungal, UV resistant, flame resistant, flame retardant, stain resistant, anti-oxidant and pigments.

14. A floor covering (20) comprising the wool-like yarn of any of claims 12 to 13, wherein the wool-like yarn (9) is tufted, knitted, knotted and/or woven and forms an upstanding pile (24).

## Patentansprüche

1. Verfahren zur Herstellung eines wollartigen Garns (9) aus Endlosfilamenten (1) aus Polymermaterial zur Verwendung als aufrechter Flor eines Bodenbelags (20), wobei das Garn durch ein Verfahren erhalten wird, das die Schritte umfasst:
- Bereitstellen von zumindest teilweise orientierten Endlosfilamenten aus dem Polymer;
- Verstrecken und Lufttexturieren der Filamente, um einen Faden (5) zu bilden, wobei eine erste Gruppe gerader Filamente einen Kern (12) des Fadens bildet und eine zweite Gruppe von Filamenten in Bezug auf die erste Gruppe von Filamenten überfüttert wird, um einen haarige Hülle (4) zu bilden;
- Verzwirnen und/oder Verdrillen einer Vielzahl von Fäden miteinander, um das wollartige Garn (9) mit einem Gewicht von mehr als 2000 dtex zu bilden.

2. Verfahren nach Anspruch 1, wobei die Vielzahl von Endlosfilamenten einen dtex-Wert pro Filament in einem Bereich von 0,5 bis 10, vorzugsweise von 4 bis 6, aufweist und/oder durch Schmelzspinnen und Verstrecken bereitgestellt wird und/oder eine multilobale Querschnittsform aufweist.

3. Verfahren nach einem der vorstehenden Ansprüche, wobei die teilweise orientierten Endlosfilamente als eine Vielzahl von Multifilament-Seilen (2) bereitgestellt werden, von denen jedes vorzugsweise einen dtex im Bereich von 100 dtex bis 1500 dtex aufweist und vorzugsweise mit Zwickstellen versehen ist, um jedes Seil zusammenzuhalten, wobei ein erstes Seil einen Kern des Fadens bildet und mindestens ein weiteres Seil zur Bildung der haarigen Hülle überfüttert wird.

4. Verfahren nach einem der vorstehenden Ansprüche, wobei das Verstrecken und die Lufttexturierung gleichzeitig in einem kontinuierlichen Prozess erfolgen.

5. Verfahren nach einem der vorstehenden Ansprüche, wobei das Verstrecken bei einer Temperatur im Bereich von 130°C - 200°C durchgeführt wird.

6. Verfahren nach einem der vorstehenden Ansprüche, wobei die zweite Gruppe von Filamenten gegenüber der ersten Gruppe von Filamenten zwischen 30% und 150 %, vorzugsweise um 80 %, überfüttert wird.

7. Verfahren nach einem der vorstehenden Ansprüche, wobei das dtex-Gewichtsverhältnis der Filamente im Kern zu den Filamenten in der Hülle zwischen 1:1 und 1:6, vorzugsweise 1:2, liegt.

8. Verfahren nach einem der vorstehenden Ansprüche, wobei der Faden einen dtex im Bereich von 500 dtex bis 5000 dtex, vorzugsweise 2000 dtex bis 3000 dtex, aufweist.

9. Verfahren nach einem der vorstehenden Ansprüche, bei dem 2 bis 20 Fäden miteinander verzwirnt und/oder verdrillt werden, um das wollähnliche Garn zu bilden, und/oder das verzwirnte und/oder verdrillte Garn in einem Bereich von 30 bis 400 Drehungen pro Meter (TPM) verzwirnt wird.

10. Verfahren nach einem der vorstehenden Ansprüche, ferner umfassend eine Thermofixierung des verzwirnten und/oder verdrillten Garns, um den Zwirn auf einer Temperatur unterhalb der Verstreckungstemperatur zu halten, vorzugsweise in einem Temperaturbereich zwischen 85°C und 110°C.

11. Verfahren nach einem der vorstehenden Ansprüche, wobei das Polymer aus der Gruppe ausgewählt ist, die aus Polyestern, Polyamiden, Polypropylen und deren Copolymeren, vorzugsweise Polyester, besteht, und/oder das Garn zu mindestens 99 % oder mindestens 95 % aus Filamenten eines einzigen Polymers besteht.

12. Wollartiges Garn (9) zur Verwendung als aufrechtstehender Flor bei der Herstellung von Bodenbelägen (20), wobei das Garn Endlosfilamente (1) aus Polymermaterial umfasst, die zu Fäden (5) zusammengefügt sind, wobei erste gerade Filamente einen Kern (12) des Fadens bilden und zweite texturierte Filamente eine haarige Hülle (4) um den Kern herum bilden, und wobei eine Vielzahl von Fäden miteinander verzwirnt und/oder verdrillt sind, um ein schweres Garn mit mehr als 2000 dtex zu bilden.

13. Wollartiges Garn nach Anspruch 12, wobei das Polymermaterial ein oder mehrere Masterbatches enthält, die aus der Gruppe ausgewählt sind, umfassend: antimikrobiell, antimykotisch, UV-beständig, flammfest, flammhemmend, schmutzabweisend, antioxidativ und Pigmente.

14. Bodenbelag (20), der das wollartige Garn nach einem der Ansprüche 12 bis 13 umfasst, wobei das wollartige Garn (9) genoppt, gewirkt, geknotet und/oder gewebt ist und einen aufrechten Flor (24) bildet.

## Revendications

1. - Procédé de fabrication d'un fil de type laine (9) à partir de filaments continus (1) de matière polymère, en vue d'une utilisation comme poil dressé d'un revêtement de sol (20), le fil étant obtenu par un procédé comprenant les étapes consistant à :
- fournir des filaments continus, au moins partiellement orientés, du polymère ;
- étirer et texturer à l'air les filaments pour former un fil (5), un premier groupe de filaments droits formant une âme (12) du fil et un second groupe de filaments étant suralimenté par rapport au premier groupe de filaments pour former une gaine velue (4) ;
- torsader et/ou câbler une pluralité de fils ensemble pour former le fil de type laine (9) ayant un poids de plus de 2000 dtex.

2. - Procédé selon la revendication 1, dans lequel les différents filaments continus ont une valeur de dtex par filament dans une plage de 0,5 à 10, de préférence de 4 à 6 et/ou sont obtenus par filage par fusion et étirage et/ou ont une forme de section transversale multilobale.

3. - Procédé selon l'une quelconque des revendications précédentes, dans lequel les filaments continus, partiellement orientés, sont fournis sous la forme d'une pluralité de paquets de multifilaments (2), chacun ayant de préférence un dtex dans une plage de 100 dtex à 1500 dtex et comportant de préférence des pincements pour maintenir chaque paquet ensemble, un premier paquet formant une âme du fil et au moins un autre paquet étant suralimenté pour former la gaine velue.

4. - Procédé selon l'une quelconque des revendications précédentes, dans lequel l'étirage et la texturation à l'air se déroulent simultanément dans un processus continu.

5. - Procédé selon l'une quelconque des revendications précédentes, dans lequel l'étirage est effectué à une température dans une plage de 130°C à 200°C.

6. - Procédé selon l'une quelconque des revendications précédentes, dans lequel le second groupe de filaments est suralimenté par rapport au premier groupe de filaments d'entre 30% et 150%, de préférence d'environ 80%.

7. - Procédé selon l'une quelconque des revendications précédentes, dans lequel un rapport en poids de dtex des filaments dans l'âme aux filaments dans la gaine est entre 1:1 et 1:6, de préférence de 1:2.

8. - Procédé selon l'une quelconque des revendications précédentes, dans lequel le fil a un dtex dans une plage de 500 dtex à 5000 dtex, de préférence de 2000 dtex à 3000 dtex.

9. - Procédé selon l'une quelconque des revendications précédentes, dans lequel de 2 à 20 fils sont torsadés et/ou câblés ensemble pour former le fil de type laine et/ou le fil torsadé et/ou câblé est torsadé dans une plage de 30 à 400 torsions par mètre (TPM).

10. - Procédé selon l'une quelconque des revendications précédentes, comprenant en outre une thermofixation du fil torsadé et/ou câblé de type laine pour maintenir la torsion à une température inférieure à la température d'étirage, de préférence dans une plage de température de 85°C à 110°C.

11. - Procédé selon l'une quelconque des revendications précédentes, dans lequel le polymère est choisi dans le groupe consistant en polyesters, polyamides, polypropylène et copolymères de ceux-ci, de préférence un polyester, et/ou le fil de type laine consiste en au moins 99% ou au moins 95% de filaments d'un seul polymère.

12. - Fil de type laine (9) en vue d'une utilisation comme poil dressé dans la fabrication de revêtements de sol (20), le fil de type laine comprenant des filaments continus (1) de matière polymère, assemblés ensemble pour former des fils (5) avec des premiers filaments droits formant une âme (12) du fil et des seconds filaments texturés formant une gaine velue (4) autour de l'âme, et dans lequel plusieurs fils sont torsadés et/ou câblés ensemble pour former un fil lourd de type laine de plus de 2000 dtex.

13. - Fil de type laine selon la revendication 12, dans lequel la matière polymère comprend un ou plusieurs mélanges-maîtres, choisis dans le groupe consistant en : antimicrobien, antifongique, résistant aux UV, ignifuge, retardateur de flamme, résistant aux taches, antioxydant et pigments.

14. - Revêtement de sol (20) comprenant le fil de type laine selon l'une quelconque des revendications 12 et 13, dans lequel le fil de type laine (9) est touffeté, tricoté, noué et/ou tissé et forme un poil dressé (24).
